

# United States Patent Office

2,745,799  
Patented May 15, 1956

1

2,745,799

## PROCESSES FOR COATING ALUMINUM AND ALLOYS THEREOF

Jos Patrie, Tournus, France, assignor to Pechiney Compagnie de Produits Chimiques et Electrométallurgiques, Paris, France, a corporation of France

No Drawing. Application March 11, 1952,  
Serial No. 276,047

Claims priority, application France March 16, 1951

10 Claims. (Cl. 204—38)

The present invention relates to the coating of aluminum and its alloys with other metals by wet methods, and, more particularly, by electrolysis after suitable preliminary treatment of the metallic surfaces to be coated.

It is known that the electrochemical coating of aluminum and its alloys involves various difficulties and that, in general, the products obtained according to the known processes present various defects, the most serious of them being: insufficient adherence, blisters, lack of homogeneity, porosity of the layer of metal deposited, sensitivity to corrosion, etc.

For example, in the commercially highly important instances of nickel and/or chromium coating, where it is generally necessary to deposit first a layer of zinc, then another layer of copper before nickel plating, the processes currently employed in the art retain the above defects. The presence of an intermediate layer of copper is largely responsible for this state of affairs.

On the other hand, when it is desired to obtain bright deposits of nickel or of chromium, it is necessary to effect several polishings, especially before coating with zinc, following coating with copper and following coating with nickel; the expense involved is considerably increased and mechanization of the treatment is made possible.

The present invention has for its object a process which makes it possible to obtain on aluminum and its alloys, sound electrolytic deposits which adhere firmly, resist corrosion well, are free from blisters or other defects and, moreover, are capable of taking a very high lustre.

According to one feature of this invention, aluminum or an alloy of this metal, after having been degreased and pickled according to a known method, is treated with an alkaline zincate solution, containing an alkali cyanide and copper cyanide. This treatment, which has for a result the formation of a highly adherent, homogeneous, fine-grained zinc deposit, can be carried out electrolytically, but it is preferable to produce it by simple immersion.

While the alkaline zincate solution may be prepared in different ways, it is best that its composition be comprehended within the following limits:

ZnO—25 to 150 grs./litre and preferably 50 to 100 gr./l.  
NaOH—100 to 600 grs./litre and preferably 250 to 350 gr./l.

KCN—30 to 170 grs./litre and preferably 130 to 170 gr./l.

CuCN—0.1 to 40 grs./litre and preferably 3 to 6 gr./l.

As is well understood, the caustic soda may be replaced by potash and the KCN by NaCN. The copper may be replaced in part or in whole by another heavy metal capable of forming a cyanide complex—i. e. a double cyanide—for example, by silver or cadmium. The concentration of the CuCN should not exceed  $\frac{1}{4}$  that of KCN.

According to a second feature of the invention, particularly favorable results are obtained when the articles

2

to be coated, having received a first treatment with an alkaline zincate, are subjected to the action of an acid which is capable of dissolving zinc and, thereafter, to a second treatment with the zincate. These various treatments are accompanied by the usual operations and rinsing.

Another feature of the process, according to the present invention, resides in the use of slightly acid nickel-plating baths having a high concentration of strong electrolytes, preferably sulfates, for nickel-plating electrolytically the articles which have been zinc-plated in accordance with the above described method.

Baths having the following compositions can be used successfully:

|                                                     | Gr./litre  |
|-----------------------------------------------------|------------|
| NiSO <sub>4</sub> .7H <sub>2</sub> O                | 70 to 140  |
| H <sub>3</sub> BO <sub>3</sub>                      | 10 to 50   |
| NH <sub>4</sub> Cl or NaCl                          | 10 to 30   |
| Na <sub>2</sub> SO <sub>4</sub> .10H <sub>2</sub> O | 200 to 450 |

20 The sodium sulfate can be replaced in part or in whole by the corresponding salt of potassium, lithium, or of magnesium, but the molecular concentration of the strong electrolyte must always be greater than that of the nickel salt used.

25 These baths, having a pH between 5 and 5.6, can be used at temperatures between 15° and 40° C., or preferably, between 20° and 35° C. and with a current density of 1 to 4 amp./dm.<sup>2</sup>. Under these conditions, there are obtained fine-grained, highly adherent nickel deposits of a quality impossible to obtain by the known methods on aluminum and its alloys. It is remarkable that the process gives excellent results even in the case of alloys which, in general, are difficult to coat by electrodeposition as is true, for example, in the case of Al-Mg alloys.

30 The nickel deposits obtained in the manner described above, have, moreover, the advantage of not requiring laborious treatments, polishings, etc., when it is desired to cover them with a bright chromium layer. In contrast with the practices of the prior art, it is sufficient, when proceeding in accordance with the present invention, to lightly "burnish," i. e. "color" (which terms are used here and in the appended claims to designate the last

35 stage of a polishing treatment) the nickel layer before it is chromium plated; there are obtained in this way, deposits of chromium which have a bright decorative appearance. Moreover, in the case of articles of simple shape, the "coloring" (burnishing) of the nickel layer is not even necessary and the chromium plating can take place immediately.

40 According to another feature of the invention, articles of aluminum or aluminum alloys can receive a bright deposit of electrolytic nickel having a strength and lustre superior to those obtained by the known methods and, in particular, by the electrodeposition of a bright nickel layer on a underlying layer of copper. According to this particular feature of the present invention, the bright nickel layer is deposited in the presence of brightening agents in accordance with known techniques (for example, those described in the U. S. Patents Nos. 2,191,813; 2,238,861; 2,523,190; 2,523,191; 2,402,801; etc.) on a primary electrolytic deposit of nickel obtained, in accordance with the previously mentioned features of the present invention, in a bath having a high sulfate content; this primary deposit is passivated by treatment with an acid, and is rinsed before being subjected to plating with a bright nickel layer.

45 If the article is to receive a chromium finish, this may be done under the usual conditions, and there is obtained a decorative chromium plating of very high quality.

50 The zinc plating of aluminum or its alloys with an

alkaline zincate solution in the presence of an alkali cyanide and of a heavy metal capable of forming a cyanide complex—i. e. a double cyanide—constitutes, according to the present invention, a preparation of the surface to enable the deposition not only of ferrous metals, such as nickel, chromium, cobalt, but also of other metals such as cadmium, silver, gold, tin, etc. and also of alloys, such as bronze, brass, etc.

In the case of brass, particularly, when the latter has been deposited from a cyanide bath, according to a known method, on an article which has preliminarily been treated in accordance with the present invention, the highly adherent brass layer is adapted to serve as a support for other deposits. Thus, very good results are obtained by depositing on the brass-coated articles, following a simple washing operation, a bright nickel layer by a known process. If a chromium deposit be desired, it may be applied and it has the advantages previously mentioned, resulting from operating in accordance with the present invention.

#### Example 1

Articles of Duralumin (that is, an alloy of aluminum containing approximately 4% Cu, 0.6% Mg, 0.6% Mn and 0.4% Si) are degreased first, by means of trichloroethylene and then, electrolytically in a bath containing 100 grams per litre of  $Na_3PO_4$ , 20 gr./l. of  $Na_2CO_3$  and 5 gr./l. of  $Na_2SiO_3$  at 12 volts, 5 amp./dm.<sup>2</sup>, for one minute at 20° C. Following rinsing in running water, neutralization with an aqueous solution containing 15% by volume of  $H_2SO_4$ , and 5% by weight of  $H_2CrO_4$ , and washing, the articles are immersed for 30 seconds in a solution maintained at 30° C. and containing:

|      | Grammes per litre |
|------|-------------------|
| NaOH | 300               |
| ZnO  | 75                |
| CuCN | 6                 |
| KCN  | 170               |

As a result, there is formed a deposit of zinc which is washed, then dissolved in nitric acid of 40° Baumé. After being washed, the articles are again immersed in the above described zinc bath for 45 seconds at 30° C. They are then washed and subjected to electrolytic coating with nickel in a bath composed of:

|                         | Grammes |
|-------------------------|---------|
| $NiSO_4 \cdot 7H_2O$    | 110     |
| NaCl                    | 25      |
| $Na_2SO_4 \cdot 10H_2O$ | 200     |
| $H_3BO_3$               | 50      |
| Water                   | 1000    |

the pH of this bath ranging between 5.5 and 6.2. The operation is carried out at 20° C. with a current density of 1.5 amp./dm.<sup>2</sup> for 15 minutes while the solution is energetically agitated by the injection of compressed air. The thickness of the nickel deposit on the article is approximately 5 to 6 microns; it is firmly adherent, homogeneous, and fine-grained.

#### Example 2

The Duralumin articles, coated with zinc and nickel, according to Example 1, are rapidly burnished ("colored") by means of a felt disc, 30 centimeters in diameter, turning at 2000 R. P. M. They are then plated with chromium for 4 minutes at 35° C. with a current density of 12 amp./dm.<sup>2</sup> in a bath containing 300 gr. of  $H_2CrO_4$  and 3 gr. of  $H_2SO_4$  per litre. There is obtained a beautiful, solid and bright chromium coating.

#### Example 3

The treatments described in Example 1 are applied to articles made of commercial aluminum, following which the nickel surface is depassivated by dipping the articles for 2 minutes at ordinary temperatures in an aqueous solution containing 300 gr. of  $H_2SO_4$  per litre. Once

rinsed, these articles are coated with a bright nickel deposit, according to a known process, in a bath composed of 300 gr.  $NiSO_4 \cdot 7H_2O$ , 60 gr.  $NiCl_2 \cdot 6H_2O$ , 60 gr.  $H_3BO_3$ , 1000 gr. of distilled water and 10 gr. of brightening agents (described in U. S. Patent No. 2,191,813); this bright nickel plating is carried out at 55° C. with a current density of 4 amp./dm.<sup>2</sup> for 10 minutes, while the articles are agitated mechanically.

#### Example 4

An aluminum article coated with a bright nickel layer by the process described in Example 3, is washed with water and treated for 15 seconds at ordinary temperatures with an aqueous solution containing 300 gr.  $H_2SO_4$  per litre. Following rinsing, it is chromium plated in the manner indicated in Example 2.

The resultant lustre of the bright chromium layer is superior to that which is obtained by the use of known processes which include thorough polishings of the supporting layer before plating with chromium.

#### Example 5

Following degreasing and pickling in a bath containing a phosphate and carbonate of soda, articles made of an aluminum alloy containing 4.5% Si, 0.7% Mg and 0.5% Mn, are rinsed and neutralized with a solution containing 15%  $H_2SO_4$  and 5%  $H_2CrO_4$ ; they are then again washed, and are thereafter dipped for about one minute in 40° Bé. nitric acid, to which has been added 0.5% HF.

The articles are then rinsed and coated with zinc in a bath having the following composition:

|      | Gr./litre |
|------|-----------|
| NaOH | 350       |
| ZnO  | 90        |
| CuCN | 4         |
| NaCN | 100       |

The sequence of operations is the same as in Example 1 following the coating with zinc, and is completed by bright nickel plating, according to Example 3, then chromium plating in accordance with Example 4. There is obtained in this way, without resorting to any intermediate or final mechanical polishings, articles with a solid chromium coating and a high lustre.

#### Example 6

The operations described in Examples 1 and 3 are carried out on articles of an aluminum alloy containing 11% Mg, thereby producing a final nickel deposit which is bright and highly adherent.

#### Example 7

Articles of Duralumin are zinc plated twice in the alkaline zincate solution containing cyanides, the operations being carried out as set forth in Example 1; they then receive an electrolytic deposit of brass in a bath having the following composition:

|            | Gr.  |
|------------|------|
| CuCN       | 30   |
| $Zn(CN)_2$ | 8.5  |
| NaCN       | 50   |
| $Na_2CO_3$ | 30   |
| Water      | 1000 |

The operation is carried out at 35° C. with a current density of 0.5 amp./dm.<sup>2</sup>, for 2 minutes. The resulting deposit is 0.5 micron thick, and is highly adherent.

#### Example 8

Articles which have been zinc and brass plated, as in Example 7, are directly coated by a known process (Cf. U. S. Patent No. 2,191,813) with a very thick—40 microns—electrolytic deposit of bright nickel. They are well protected against corrosion by this thickness of nickel, which is very shiny and does not show any blisters or other defects.

Articles which have been zinc, brass and nickel plated, as in Example 8, are chromium plated in a bath—maintained at 35° C.—containing 300 gr. H<sub>2</sub>CrO<sub>4</sub> and 3 gr. H<sub>2</sub>SO<sub>4</sub> per litre, with a current density of 12 amps./dm.<sup>2</sup>.

I claim:

1. Process of electrolytically coating aluminum and alloys thereof with other metals comprising the steps of: zinc plating the article in an aqueous alkaline solution consisting essentially of zincate, alkali cyanide and a cyanide of a heavy metal of the group consisting of copper, silver and cadmium, wherein the ratio of weight of the alkali cyanide to the heavy metal cyanide is greater than 4, and thereafter electrically depositing a metal other than zinc.

2. A process according to claim 1, wherein the heavy metal is copper.

3. Process for electrolytically coating aluminum and alloys thereof with other metals comprising the steps of: zinc plating the aluminum by immersion in an aqueous alkaline solution consisting essentially of zincate, alkali cyanide and a proportion by weight of copper cyanide less than 1/4 that of the alkali cyanide; dissolving by an acid the layer of zinc thus formed; again zinc plating and thereafter electrolytically depositing a metal other than zinc.

4. A process according to claim 3, wherein the metal other than zinc is nickel, deposited from a bath containing, in addition to a solution of a nickel compound, a strong electrolyte in a molar concentration greater than that of the nickel compound in solution, the said bath having a pH ranging between 5 and 6.5.

5. A process according to claim 4, characterized by the additional steps of de-passivating the nickel deposited by treatment with an acid solution, and electrolytic deposition of nickel in a bath containing a brightening agent, whereby a bright nickel coating is obtained.

6. A process according to claim 4, characterized by the additional steps of burnishing the nickel deposit, and electrolytically depositing chromium thereon in a chromic acid bath containing sulfuric acid.

5 7. A process according to claim 4, characterized by the additional steps of de-passivating the nickel deposited by treatment with an acid solution, electrolytic deposition of nickel in a bath containing a brightening agent, whereby a bright nickel coating is obtained, and electrolytic deposition of chromium on the bright nickel coating in a chromic acid bath containing sulfuric acid, whereby an outer coating of bright chromium is obtained.

10 8. A process according to claim 3, wherein the metal other than zinc is brass deposited electrolytically from an alkaline bath containing an alkali cyanide and cyanides of zinc and copper.

15 9. A process according to claim 8, characterized by the additional feature of providing a bright nickel coating by electrolytically depositing the same from a bath containing a brightening agent.

20 10. A process according to claim 8, characterized by the additional features of providing a bright nickel coating by electrolytically depositing the same from a bath containing a brightening agent, and thereafter chromium plating electrolytically the nickel coating in a chromic acid bath containing sulfuric acid.

#### References Cited in the file of this patent

#### UNITED STATES PATENTS

|    |           |               |       |               |
|----|-----------|---------------|-------|---------------|
| 30 | 1,405,534 | Merritt       | ----- | Feb. 7, 1922  |
|    | 2,091,386 | Viers         | ----- | Aug. 31, 1937 |
|    | 2,142,564 | Korpiun       | ----- | Jan. 3, 1939  |
|    | 2,418,265 | Korpiun       | ----- | Apr. 1, 1947  |
| 35 | 2,496,845 | Balden et al. | ----- | Feb. 7, 1950  |
|    | 2,650,902 | Higgins       | ----- | Sept. 1, 1953 |
|    | 2,662,054 | Passal        | ----- | Dec. 8, 1953  |